# EUROPEAN PATENT SPECIFICATION

(11) **EP 4 204 617 B1**
(45) Date of publication and mention of the grant of the patent: **12.03.2025**
(21) Application number: 21937194.5
(22) Date of filing: 30.11.2021
(51) Int. Cl.: D04B 21/00, D01G 11/04, D03D 13/00, D03D 15/217, D03D 15/47

(54) **A FLANNEL FABRIC PRODUCTION METHOD UTILIZING END-USER'S WASTE FABRIC**
VERFAHREN ZUR HERSTELLUNG VON SCHLANNELGEWEBE UNTER VERWENDUNG VON GEBRAUCHTGEWEBE FÜR ENDBENUTZER
PROCÉDÉ DE PRODUCTION DE TISSU DE FLANELLE UTILISANT DES DÉCHETS DE TISSU D'UTILISATEUR FINAL

(30) Priority: 22.11.2021 TR 202118222
(43) Date of publication of application: 05.07.2023
(73) Proprietor: MENDERES TEKSTIL SANAYI VE TIC. A.S., Denizli (TR)
(72) Inventor: KAYMAKCI, Serdar, Sarayköy/Denizli (TR); ALSAN, Serkan, Sarayköy/Denizli (TR); GÜNGÖR, Yusuf, Sarayköy/Denizli (TR); KARAOGLU, Fatma, Sarayköy/Denizli (TR); GÖDE, Ceren, Sarayköy/Denizli (TR); ERTUNA, Süleyman Ilker, Sarayköy/Denizli (TR)
(74) Representative: Valet Patent Services Limited
(86) International application number: PCT/TR2021/051315
(87) International publication number: WO 2023/091102

(56) References cited:
- CN-A- 105 369 450
- CN-A- 105 420 887
- CN-A- 105 420 891
- CN-A- 112 176 461
- CN-B- 104 562 715
- US-A1- 2011 250 425

## Description

### TECHNICAL FIELD

The invention relates to a flannel fabric production method which enables utilizing waste fabric owned by end-user, incentivizing the end-user by way of rewards, eliminating the need for waste sorting and thereby preventing loss of productivity and time, and converting the waste fabric owned by the end-user into the flannel fabric, a product with high added-value, and thus preventing loss and waste.

### BACKGROUND ART

CN 104 562 715 B describes a flannel fabric production method which comprises obtaining wefts of 28.1 tex (Ne 21) and warps of 28.1 tex (Ne 21) from a drawing process and obtaining a woven fabric having a weft density of 30.7 ends/centimeter and a warp density of 26.8 ends/centimeter and turning the woven fabric into flannel by napping it in a raising process.

Today, end users' waste products such as paper, plastic, metal, fabric, and the like are collected with various methods for recycling purposes. These collected waste products contain different materials therein since they are typically not sorted, and this leads to a reduction in the quality of yarns obtained from these waste products and of the fabric produced with such yarns. CN 112 176 461 A and US 2011/250425 A1 disclose methods for recycling cotton fibres and processing these fibres into yarns.

Due to the reasons explained hereinabove, in order to manufacture flannel fabric, 100% cotton waste products should be collected from the end-user and should be worked on.

In conclusion, the abovementioned shortcomings and the inadequacy of the current practice entail an improvement in the respective technical field. Thus, there is a need for an invention to overcome the described problems.

### OBJECTIVE OF THE INVENTION

Developed for eliminating the aforementioned disadvantages and providing new advantages to the respective technical field, the present invention relates to a flannel fabric production method utilizing the end-user's waste fabric.

The objectives of the present invention can be listed as follows: to obtain new fabric by utilizing the end user's waste fabrics and thereby convert wastes into a product with high added-value, to provide an opportunity to obtain flannel fabric by way of recycling, to reward the end-user by collecting waste fabric at stores and thus incentivize the end-user for the collection of waste fabric, to eliminate the need for waste sorting and thus achieve saving on expenses and time, to prevent waste by utilizing waste fabrics, to provide fabric to be recycled during this period of cotton supply shortage, and to obtain quality fabrics from waste fabrics. Structural and characteristic features of the invention, as well as all of its advantages, will be understood more clearly with the detailed description provided below, and therefore, the evaluation should be made by taking into consideration of the said detailed description.

### DETAILED EXPLANATION OF THE INVENTION

The preferred alternatives in this detailed description of the method of the present invention are only intended for providing a better understanding of the subject matter and should not be construed in any restrictive sense.

The invention relates to a flannel fabric production method which enables utilizing waste fabric owned by the end-user, incentivizing the end-user by way of rewards, eliminating the need for waste sorting and thereby preventing loss of productivity and time, and converting the waste fabric owned by the end-user into the flannel fabric, a product with high added-value, and thus preventing loss and waste.

The method of the present invention consists of the following process steps: collecting end user's waste cotton products at stores by way of campaigns for eliminating the need to sort wastes, converting the collected waste cotton products into fiber at fiber opening facility, blending the recycled fiber and the virgin cotton at a rate of 30% and 70%, respectively, in regard to the total blend amount, obtaining wefts of 73.8 tex (Ne 8/1) and warps of 29.5 tex (Ne 20/1) from the blend by drawing process and obtaining fabric having weft density of 13.5 ends/centimeter and warp density of 20 ends/centimeter by way of weaving the threads, and turning the woven fabric into flannel by napping it through raising process.

Being the first endeavor in terms of obtaining flannel fabric from recycled material, the method of the present invention prevents losses relating to cotton and reproduction and recovers waste products by way of recycling waste cotton materials owned by the end-users. The obtained flannel fabric is distinguished in that it is eco-friendly and is manufactured from end user's waste. The obtained flannel fabric has a structure suitable for all dyeing processes except for digital printing.

## Claims

1. A flannel fabric production method which enables utilizing waste fabric owned by end-user, incentivizing the end-user by way of rewards, eliminating the need for waste sorting, and converting the waste fabric owned by the end-user into the flannel fabric, the method consisting of the following process steps:
- collecting the end user's waste cotton products at stores by way of campaigns for eliminating the need to sort wastes;
- converting the collected waste cotton products into fiber at fiber opening facility;
- blending the recycled fiber and virgin cotton at a rate of 30% and 70%, respectively, in regard to the total blend amount;
- obtaining wefts of 73.8 tex (Ne 8/1) and warps of 29.5 tex (Ne 20/1) from the blend by drawing process and obtaining fabric having weft density of 13.5 ends/centimeter and warp density of 20 ends/centimeter by way of weaving the threads; and
- turning the woven fabric into flannel by napping it through raising process.

## Patentansprüche

1. Verfahren zur Herstellung von Flanellstoffen, das es ermöglicht, Stoffabfälle von Endverbrauchern zu verwenden, den Endverbraucher durch Belohnungen zu motivieren, die Notwendigkeit der Abfalltrennung zu eliminieren und die Stoffabfälle der Endverbraucher in Flanellstoffe umzuwandeln, das Verfahren, das aus den folgenden Prozessschritten besteht:
- Sammlung der Abfälle von Baumwollprodukten des Endverbrauchers in Geschäften durch Kampagnen, um die Notwendigkeit der Abfalltrennung zu eliminieren;
- Umwandlung der gesammelten Abfälle von Baumwollprodukten in Fasern in einer Faseröffnungsanlage;
- Mischung der recycelten Faser und der neuen Baumwolle in einem Verhältnis von jeweils 30% und 70% in Bezug auf die gesamte Mischungsmenge;
- Gewinnung von Schussfäden mit 73,8 tex (Ne 8/1) und Kettfäden mit 29,5 tex (Ne 20/1) aus der Mischung durch den Ziehprozess sowie die Gewinnung von Stoffen mit einer Schussfadendichte von 13,5 Enden/Zentimeter und einer Kettfadendichte von 20 Enden/Zentimeter durch das Weben der Garne; und
- Verwandlung des gewebten Stoffes in Flanell durch Aufrauen im Rauprozess.

## Revendications

1. Procédé de production de tissu en flanelle qui permet d'utiliser des déchets de tissu appartenant à un utilisateur final, d'inciter l'utilisateur final par le biais de récompenses, de supprimer le besoin de trier les déchets, et de convertir les déchets de tissu appartenant à l'utilisateur final en tissu en flanelle, le procédé étant constitué des étapes de processus suivantes :
- la collecte de produits déchets de coton de l'utilisateur final dans des magasins par le biais de campagnes de suppression du besoin de trier les déchets ;
- la conversion des produits déchets de coton collectés en fibre dans une installation d'ouverture de fibre ;
- le mélange de la fibre recyclée et de coton vierge selon un taux de 30 % et 70 %, respectivement, par rapport à la quantité totale de mélange ;
- l'obtention de trames de 73,8 tex (Ne 8/1) et de chaînes de 29,5 tex (Ne 20/1) à partir du mélange par un processus d'étirage et l'obtention d'un tissu ayant une densité de trames de 13,5 extrémités/centimètre et une densité de chaînes de 20 extrémités/centimètre par le biais d'un tissage des fils ; et
- la transformation du tissu tissé en flanelle en le grattant au moyen d'un processus de lainage.
